# EUROPEAN PATENT APPLICATION

(11) **EP 0 559 539 A1**
(43) Date of publication of application: **08.09.1993**
(21) Application number: 93400514.1
(22) Date of filing: 01.03.1993
(51) Int. Cl.: B21B 1/08

(54) **Process for manufacturing H-shaped steels**

(30) Priority: 02.03.1992 JP 44934/92
(71) Applicant: SUMITOMO METAL INDUSTRIES, LTD., Osaka-Shi Osaka 541 (JP)
(72) Inventor: Shikano, Hiroshi 404 Daiichi-Takamagahara-Shataku, Kashima-gun, Ibaraki-ken (JP)
(74) Representative: Schrimpf, Robert

(57) **Abstract**

A process for manufacturing H-shaped steels through intermediate hot rolling, and finishing hot rolling to provide H-shaped steels is disclosed. The horizontal roll is divided into two or more pieces in a roll axis direction, the width is adjustable for each pass. The intermediate rolling comprises a first step of forming one or more non-rolled portions on the surface of the web while carrying out reduction in web thickness as well as reduction in the thickness of flanges; a second step of flattening the web surface to expand the inner web width while not only reduction in thickness of the flange but also reduction in thickness of the web are carried out with the other universal mill; alternatively a first step of flattening the web surface while performing reduction in flange thickness with one of the first and second universal mills; a second step of forming one or more non-rolled portions on the web surface and simultaneously reducing the inner web width while not only reduction in thickness of the flange but also reduction in thickness of the web are carried out with the other universal roughing mill; and repeating the first and second steps until a predetermined amount of expansion or reduction is achieved.

## Description

The present invention relates to a process for manufacturing H-shaped steels, such as H-shaped beams and H-shaped piles, for use in civil engineering and the construction industry, and in particular to a process for manufacturing, through hot rolling, H-shaped steels having various sizes of high quality in the same rolling chance using the same rolls without changing the rolls, resulting in a high efficiency and high yield of H-shaped steels with a marked reduction in the number of rolls to be retained.

Generally, a conventional rolling mill line for producing H-shaped beams and channels comprises, as shown in Figure 4a, three different types of mills: a breakdown mill (hereunder referred to as a "BD-mill") 10, a universal roughing mill (hereunder referred to as a "UR-mill") 11, an edging mill (hereunder referred to as an "E-mill") 12, and a universal finishing mill (hereunder referred to as a "UF-mill") 13. The BD-mill, UR-mill + E-mill, and UF-mill are arranged in a tandem line in this order. A rolling material, such as slabs, rectangular steel pieces, and blank beams, is rough rolled with the breakdown mill 10 to give a predetermined rough shape, then through intermediate reverse rolling with the universal roughing mill 11 and edging mill 12 a rolling workpiece having the rough shape is further rolled to give a predetermined final shape and is finished with a universal finishing mill 13 to obtain a final product.

Figure 5a shows a rolling process in which a web 2 of the H-shaped steel is rolled with a pair of horizontal rolls 20 of the UR-mill 11 while flanges 1a, 1b are supported with a pair of tapered vertical rolls 21. The top and bottom ends of flanges 1a, 1b are reduced in height with a pair of edging rolls 22 of the E-mill 12. Rolling with the UR-mills 11 and the E-mill 12 is repeated. As a result of the rolling with the UF-mill 13, the flanges 1a, 1b are made upright by the action of horizontal rolls 23 and vertical rolls 24.

As an efficient method for rolling H-shaped steels, Japanese Patent Publication No.50-21984/1975 discloses a method for rolling H-shaped steels using a mill arrangement in which an edging mill is placed between two universal roughing mills, and these three mills are arranged in a tandem line. Thus, a rolling work piece after breakdown rolling is subjected to reverse rolling by the two universal roughing mills and the edging mill before being finished with the finishing universal mill.

The mill arrangement of that publication is shown in Figure 4b, and the rolling process of the universal mill is shown in Figure 5b. A rolling material, after being rough rolled with the breakdown mill 10, is subjected to reverse rolling with the first universal roughing mill 11, the edging mill 12, and the second universal roughing mill 14, and then is finished with a universal finishing mill 13 to provide a final product.

In the roll arrangement shown in Figure 4c, in which a universal finishing mill is used in place of the second universal finishing mill of Figure 4b, the reverse rolling is carried out by the first universal roughing mill, the edging mill, and the universal finishing mill, and then the resulting H-shaped steel is finished by a final pass with the universal finishing mill making the flanges upright to provide a final product. Figure 5c shows the rolling process of this case.

Figure 4d shows still another example in which the rolling mill arrangement comprises a series of rolling mill groups in a tandem line, each group comprising an edging mill between two universal rolling mills. According to this roll mill arrangement, after roughing rolling, a rolling work piece is, in a single pass, rolled through intermediate rolling and finishing rolling to provide a final product.

In the conventional process, the size of rolls for the universal finishing mill as well as for preceding mills is determined by the size of final products.

Namely, in the roll arrangements shown in Figures 6 and 7, for example, the widths a₁ in Figure 6a and a₂ in Figure 7a, and a₃ in Figure 7b and a₄ in Figure 7c are designed to be substantially the same.

Thus, horizontal rolls of rolling mills after a breakdown rolling mill must have specific widths, and the horizontal rolls must be changed depending on the size of final products. This means that horizontal rolls having specific widths must be used for rolling a specific series of H-shaped steels (e.g., H600X300), resulting in a fixed dimension of inner web length with a varied dimension of web height. Usually the difference in flange thickness between the maximum and minimum is about 15 mm, and the web height will vary in a range of about 30 mm. It is therefore inevitable that the web height will vary even within the same series of rolled steel member. This is a serious defect when H-steels are used in the construction of buildings. Namely, when connecting several H-shaped beams of the same series (H600X300, for example), since the outer dimensions are different from each other, it is impossible to join them smoothly around the periphery. If one side is matched, the opposite sides will be apart, by double the difference in the flange thickness.

Usually when a building is designed, measurements are determined first for outside of the building and then for the inside. However, an H-shaped beam has a web having a fixed width and a varying web height. This will cause a serious problem when precise dimensions are required in a limited space.

Furthermore, the dimensions of H-shaped steels are sometimes not accurate. Namely, in a conventional rolling process, as shown in Figure 8, the vertical surfaces of horizontal rolls 82 of a universal roughing mill 80 are worn out after a substantial number of work pieces are rolled, resulting in a decrease in the width of the horizontal rolls 82. Although the vertical surfaces of vertical rolls 84 are also worn out, in order to compensate for wear of the vertical rolls, it is only necessary to adjust the position of each of the vertical rolls, i.e., to adjust the distance between the opposing vertical rolls.

When wear of horizontal rolls occurs, the web height is decreased by an amount corresponding to the amount of wear of the vertical surfaces of the horizontal rolls, provided that the thickness of flange is not varied. See Figure 9. In order to avoid a decrease in the web height of the final product, the thickness of flange is adjusted to be as thick as possible within dimensional tolerances. However, setting the flange thickness in this manner has the following disadvantages.

According to JIS G 3192, dimensional tolerances for the web height are ±3.0 mm for a web height of less than 400 mm, ±4.0 mm for a web height of 400 - 600 mm, and ±5.0 mm for a web height of 600 mm or larger. Since the web height is influenced by the width of the horizontal rolls, the horizontal rolls to be used must be chosen within the dimensional tolerances taking into consideration a target web height. This means that the thickness of the flange is determined by the width of the horizontal roll. Thus, when horizontal rolls which are worn out on the vertical surfaces are employed, the thickness of the resulting H-shaped steels is thickened. In this case, since the length extended by rolling is decreased, the yield rate of rolling is decreased, too. In addition, a variation in the dimensions of final products in different rolling chances in which the width of horizontal rolls is varied is inevitable, and a variation in flange thickness even in the same rolling chance is inevitable due to wear of the horizontal rolls. These variations in dimensions are undesirable from the viewpoint of manufacturing H-shaped steels having accurate dimensions.

In addition, when the rolling temperature in the universal finishing mill is varied, shrinkage during being cooled to room temperature after finish rolling will vary depending on the finishing temperature, resulting in a variation in dimensions in the longitudinal direction and the web height of the final product.

Since H-shaped beams produced by hot rolling have such disadvantages, sometimes H-shaped steels for use in constructing buildings are produced by welding steel plates having predetermined thicknesses to give a predetermined constant web height. However, an increase in manufacturing costs is inevitable.

In the prior art, in order to cope with such disadvantages, the following rolling methods have been proposed.

(1) A method of expanding the web height during universal rolling in order to produce H-shaped beams having different web heights by using the same rolls.

According to the rolling method disclosed in Japanese Patent Publication No.3-8841/1991, reverse rolling is carried out between at least one universal mill, the horizontal rolls of which have recesses at their edges, and at least one universal mill, the horizontal rolls of which are flat or convex at their edges. Rough rolling is finished to form swelled portions having a predetermined height at both edges of the web. The swelled portions are rolled with a rolling mill the horizontal rolls of which have flat surfaces or convex surfaces at both edges, just before finishing rolling, to provide an expansion of the inner web length. The finish rolling is then carried out using width-variable horizontal rolls.

According to this method, the expansion of the inner web length, i.e., web width is carried out with a single pass through a universal mill just before going into a finishing mill, the maximum expansion of the web width is around 30 mm, and it is rather difficult to expand the web width more than this without resulting in waviness on the web surfaces. In addition, when the web thickness is rather small, the temperature of the web is decreased to a relatively low temperature during the reverse rolling because of the cooling effect of rolls and cooling water. Thus, even when the swelled portions are rolled in a final pass, it is rather difficult to achieve expansion of the web width, and an increase in rolling loads on the horizontal rolls is inevitable. In this method, therefore, it is possible to manufacture a series of H-shaped steels having a fixed size for web height, but this method is not able to manufacture H-shaped steels having varied web height using the same rolls. It is impossible to manufacture a plurality of series of H-shaped steels, the series differing by pitches of 50 mm according to JIS Standards, in the same rolling chance without changing the rolls.

Japanese Unexamined Laid-Open Specification No.63-260602/1988 discloses a method of expanding the web width little by little by carrying out reverse rolling using just a pair of horizontal rolls each divided into two pieces which are movable along an axial direction. However, this method is not intended to expand the web width significantly, but merely to flatten an excess metal portion formed in a transitional area between a flange and web. Thus, an expansion of the web height (web width) per pass is small, and an increased number of passes must be performed when a relatively large degree of expansion (about 30 mm, for example) is required, resulting in a degradation in rolling efficiency. Furthermore, if a large rolling reduction is tried so as to attain a large expansion per pass, projections or roll marks are formed on the web in areas corresponding to a space between the two divided pieces of horizontal rolls. The presence of such defects degrades the appearance of final products. When the thickness of the web is small, the formation of local necking is inevitable. There is no measure to solve such problems.

(2) A method of reducing a web height during universal rolling in order to manufacture H-shaped steels having varied web heights using the same rolls.

Japanese Unexamined Laid-Open Specification No.2-6001/1990 discloses a rolling method for shaped steels in which a rolling process through a breakdown mill and universal roughing mill is the same as in the conventional process, but a universal finishing mill employs variable-width horizontal rolls. When an H-shaped steel is passed through the universal finishing mill, the web of a shaped steel is reduced in a width direction to produce a shaped steel having a predetermined web height.

However, during reduction of the web width buckling is inevitable, resulting in a deviation of the position of a web from the center line of the flange, i.e., web off-center. Sometimes, the buckling remains in the web in a central area corresponding to a space between the divided pieces of the horizontal rolls, and these products cannot be put on the market.

Thus, a maximum reducible width is about 30 mm in this method, and it is impossible to produce a variety of H-shaped steels having various sizes of web height in the same rolling chance without changing rolls.

(3) A method of hot rolling H-shaped steels having various sizes of web height without changing rolls, in which universal mills and edging mill having variable-width horizontal rolls each divided into two or three pieces are used.

According to a method disclosed in Japanese Unexamined Laid-Open Specification No.59-133902, as shown in Figure 10, variable-width horizontal rolls are installed in each of a universal roughing mill (UR), edging mill (E), and universal finishing mill (UF). Through this roll mill arrangement, a web 101 is partially rolled and edges of flanges 102 are rolled, making it possible to roll H-shaped steels having varied web heights using the same rolls. The width of each of the horizontal divided rolls 103, 104, and 105 is previously adjusted to a predetermined one and is not adjusted for each pass. Thus, it is necessary to previously determine the width of each of the horizontal rolls depending on the dimensions of a workpiece after breakdown rolling. This means that expansion or reduction of the web width does not take place during universal rolling. Thus, in order to produce H-shaped steels having different sizes of web height without changing rolls, it is necessary to change grooved rolls of the breakdown mill 60, as shown in Figures 6a and 6b. There is no disclosure about how to manufacture H-shaped steels having any desired web height.

Furthermore, according to this method, waviness occurs easily in the web portion during edging rolling, especially during edging rolling of a .thin web, making this process less practical. This is because there will occur a difference in elongation upon rolling between the web and flanges.

Japanese Unexamined Laid-Open Specification No.60-82201/1985 disclosed a method of rolling H-shaped steels having different web heights and flange widths without changing rolls, in which, as shown in Figure 11, variable-width horizontal rolls are installed in each of a first universal roughing mill (UR1), an edging mill (E), a second universal roughing mill (UR2), and a universal finishing mill (UF). Through this roll mill arrangement, a web 101 is partially rolled and edges of flanges 102 are rolled, making it possible to roll H-shaped steels having varied web heights using the same rolls. The width of each of the divided horizontal rolls is previously adjusted to a predetermined value and is not adjusted for each pass. Thus, it is also necessary to determine the width of each of the horizontal rolls previously depending on the dimensions of a workpiece after breakdown rolling. In order to produce H-shaped steels having different sizes of web height without changing rolls, it is necessary to change grooved rolls of the breakdown mill 60, as shown in Figures 6a and 6b. However, there is no disclosure in that publication about how to manufacture H-shaped steels having any desired web height.

Japanese Unexamined Laid-Open Specification No.61-283401/1986 discloses, as shown in Figure 12, a method of rolling a shaped steel using a mill arrangement in which each of the horizontal rolls of a universal roughing mill (UR1) is divided into two pieces to have a variable-width in a roll axis direction. A web 101 of the shaped steel is partially rolled with UR1, and then only flanges 102 are rolled with an edging mill (E), which has also divided horizontal rolls. In a universal rolling mill (UR2) a non-rolled portion on the web 101 is rolled with the horizontal rolls of UR2.

The width of each of the divided horizontal rolls is adjusted to a predetermined length previously, but is not varied for each pass during rolling with each of the mills. The width of each of the roll mills will be determined based on the dimensions of a workpiece after breakdown rolling. Thus, the web width is not expanded or reduced during rolling after breakdown rolling. In order to produce H-shaped steels having different web heights without changing rolls, it is, therefore, necessary to change grooved rolls of the breakdown mill. There is no disclosure in that publication about how to manufacture H-shaped steels having any desired web height.

In general, the prior art, in which the barrel length of each of the horizontal rolls of a universal mill and edging mill is fixed, has the following disadvantages.
i) Since final products of different series or those having different sizes cannot be manufactured in the same rolling chance without changing rolls, new series of products all of which have the same outer length, i.e., web height cannot be manufactured.
ii) The number of rolls to be stocked in the factory is huge.
iii)Since it is necessary to change rolls before rolling, rolling efficiency and operating efficiency are lowered markedly when a small lot of workpieces is rolled to manufacture a lot of products having a variety of sizes.
iv) Due to wear during rolling, the dimensions of a final product are not accurate and vary to some extent.
v) The rolling yield is very small.
vi) Since the same rolls cannot be used repeatedly for a long period of time for rolling products of the same size, roll costs are very high.

In order to solve such prior art disadvantages, the techniques in the above paragraphs (1) through (3) have been proposed. However, even in such processes, the following disadvantages are inevitable.
(i) A maximum expansion or reduction in the inner web width, which can be achieved with a universal rolling mill using the same rolls, is 30 mm.
(ii)When H-shaped steels having a thin web are rolled, necking of a web portion during expansion of inner web width and buckling of the web surface during reduction in the inner web width are inevitable if the expansion or reduction in inner web width is excessive.
   Furthermore, the prior art described in paragraphs (1) and (2) have also the following disadvantages, although H-shaped steels having the same outer length, i.e., web height can be manufactured.
(iii)It is impossible to produce H-shaped steels having any desired web height in a different series in one rolling chance without changing rolls, since a wide range of adjustment for web height is not possible without changing rolls. Namely, JIS defines the dimensions of a series of H-shaped steels with a pitch of 50 mm, and it is impossible to manufacture these series of H-shaped steels in one chance of rolling without changing rolls.
   In addition, according to the prior art described in paragraph (3) above, since expansion or reduction in an inner web width does not takes place during universal rolling, a small number of horizontal rolls can be cut for the universal rolling mill and edging mills. However, the following disadvantage still remains.
(iv)It is necessary to change grooved rolls of a breakdown mill in order to manufacture H-shaped steels having different web heights without changing rolls of universal mills and edging mill. The number of grooved rolls to be stocked is not reduced at all.

### SUMMARY OF THE INVENTION

An object of the present invention is to provide a process for manufacturing, through hot rolling, high quality H-shaped steels having various sizes in the same rolling chance using the same rolls without changing the size of the rolls.

Another object of the present invention is to provide a process for manufacturing, through hot rolling, H-shaped steels with which highly efficient rolling can be achieved with a high yield and with which the inventory of rolls can also be reduced markedly.

The present invention is a process for manufacturing H-shaped steels through intermediate hot rolling and finishing hot rolling, in which a horizontal roll employed is divided into two or more pieces in a roll axis direction, the width is adjustable for each pass, the intermediate rolling comprising a first step of forming one or more non-rolled portions on the surface of the web while carrying out reduction in web thickness as well as reduction in the thickness of flanges; a second step of flattening the web surface to expand the inner web width while not only reduction in thickness of the flange but also reduction in thickness of the web are carried out with the other universal mill or with a universal mill on the downstream side; alternatively a first step of flattening the web surface while performing reduction in flange thickness with one of the first and second universal mills; a second step of forming one or more non-rolled portions on the web surface to reduce the inner web width while not only reduction in thickness of the flange but also reduction in thickness of the web are carried out with the other universal mill or with a universal mill on the downstream side; and repeating the first and second steps until a predetermined amount of expansion or reduction is achieved.

### BRIEF DESCRIPTION OF THE DRAWINGS

Figures 1a - 1c are schematic sectional views illustrating how to expand the inner web width in accordance with the present invention.

Figures 2a - 2c are schematic sectional views illustrating how to reduce the inner web width in accordance with the present invention.

Figures 3a and 3b are schematic sectional views illustrating another example of how to reduce the inner web width in accordance with the present invention and that of the prior art, respectively.

Figures 4a - 4d are illustrations of rolling mill arrangements with which hot rolling of H-shaped steels of the prior art as well as of the present invention can be performed.

Figures 5a - 5c are schematic views illustrating a process of hot rolling in accordance with the prior art.

Figures 6a and 6b are schematic sectional views of a grooved roll of a breakdown mill.

Figures 7a - 7c are schematic views illustrating a process of hot rolling in accordance with another example of the prior art.

Figure 8 is a schematic view illustrating wear of the lateral surfaces of horizontal rolls of a conventional universal mill.

Figure 9 is a schematic illustration showing names of elements of an H-shaped steel.

Figure 10 is a schematic view illustrating a change in section of a workpiece when the web height is adjusted in accordance with the prior art.

Figure 11 is a schematic view illustrating a change in section of a workpiece when the web height is adjusted in accordance with another example of the prior art.

Figure 12 is a schematic view illustrating a change in section of a workpiece when the web height is adjusted in accordance with still another example of the prior art.

Figure 13 is a schematic view illustrating a change in section of a workpiece in each of the rolling steps when the web height is adjusted in accordance with the process of Example 1 of the present invention.

Figure 14 is a schematic view illustrating a change in section of a workpiece in each of the rolling steps when the web height is adjusted in accordance with the process of Example 2 of the present invention.

Figure 15 is a schematic view illustrating a change in section of a workpiece in each of the rolling steps when the web height is adjusted in accordance with the process of Example 3 of the present invention.

### DESCRIPTION OF PREFERRED EMBODIMENTS OF THE INVENTION

Using a first universal mill, an edging mill, and a second universal mill arranged as shown in Figure 4b, a large number of rolling simulation tests were conducted.

As shown in Figure 11, the first and second universal mill had horizontal rolls which were each divided into two or three pieces, and the edging mill also had horizontal rolls which were each divided into two pieces. The width of each of the horizontal rolls could be adjusted while the mill is on line, i.e., after or before each pass, in the roll axis direction in accordance with the inner web width of a workpiece to be rolled.

Another series of simulation tests was carried out using a first universal mill, an edging mill, and a second universal mill, which are schematically illustrated in Figure 12. In this case the horizontal roll of the universal mill was divided into two pieces. The width of each of the horizontal rolls is adjustable for each pass.

The above-described tests produced the following results.
(1) When an H-shaped steel is rolled to reduce the thickness of a flange 1 as well as of a web 2 through either one of the universal mills which have the variable-width horizontal rolls, it is desirable that, as shown in the upper each of Figures 1a - 1c, one or more non-rolled portions, i.e., projections 2a be left on the surface of the web 2 while the width of the horizontal roll is adjusted to be Wa1, Wb1, and Wc1, respectively. After rolling with this mill, reduction in thickness of the web and flange is carried out with the other universal mill which has variable-width horizontal rolls 20' so as to flatten not only the non-rolled portions 2a but also the overall surface of the web 2. The non-rolled portions 2a illustrated by phantom lines disappear. Each of widths Wa2, Wb2, and Wc2 of the horizontal roll 20' is set to be wider than Wa1, Wb1, and Wc1, respectively.
   According to this embodiment, expansion of the inner web width can be carried out easily when the workpiece is rolled in the following universal mill. From a few percent to about 15 percent expansion of the web width is possible depending on the volume of the non-rolled portions (thickness, width, and numbers) preformed on the surface of the web. The expansion ratio can be determined, for example, by the formula (Wa2 - Wa1)/(Wa1) X100 (%). The surfaces of the web and the inner surfaces of the flanges are free from rolling flaws and waviness.
(2) Furthermore, as indicated by arrows in Figures 1a - 1c, when the web width expansion rolling is carried out repeatedly using two universal mills, it is possible to expand the inner web width by 20% - 50% relative to the dimensions of a workpiece after breakdown rolling. It is advisable to carry out expansion of the web width in the first half of passes while the thickness of a web is relatively large and the temperature of the workpiece is relatively high in order to achieve a large degree of expansion as well as to finish a thin web.

The following is a case in which the web width is reduced during rolling with a universal mill.
(1) When an H-shaped steel is rolled with one of the universal mills which have variable-width horizontal rolls 20, it is desirable that not only reduction of one or more non-rolled portions, i.e, projections 2a which have been formed in the preceding rolling step on the surface of the web 2 but also reduction of flanges 1 be carried out to flatten the web surfaces, as shown in the upper portions of Figures 2a - 2c,. The width of the horizontal roll 20 is adjusted to be Wa1, Wb1, and Wc1, respectively. After being rolled with this mill, the outer surfaces of the flanges are pressed by vertical rolls of the other universal mill so as to reduce not only the inner web width but also the thickness of the flanges. Simultaneously, with the variable-width horizontal rolls 20' of this universal mill, the thickness of the web 2 is reduced until one or more non-rolled portions 2a are formed on the surface of the web 2. Each of the widths Wa2, Wb2, and Wc2 of the horizontal roll 20' is set to be narrower than Wa1, Wb1, and Wc1, respectively, of the horizontal rolls 20 of the preceding universal mill.
   According to this embodiment, reduction in the inner width of the web can be carried out easily when the workpiece is rolled in the following universal mill. From a few percent to about 15 percent reduction of the web width is possible depending on the volume of the non-rolled portions (thickness, width, and numbers) preformed on the surface of the web. The reduction ratio can be determined, for example, by the formula (Wa2 - Wa1)/(Wa1) X100 (%). The surfaces of the web and the inner surfaces of the flanges are free from rolling flaws and waviness. The dimensions of a final product are very accurate and are free from web off-center, i.e., deviation of web from the center of the flange.
   In this respect, according to the prior art, as illustrated in Figure 3b, when a universal mill having flat horizontal rolls is used, occurrence of buckling is inevitable during rolling, which causes web off-center, i.e., deviation of web position from the center of flange. In contrast, when a universal mill having divided horizontal roll is used to reduce the inner web width in accordance with the present invention, as shown in Figure 3a, the presence of tensile stresses applied in the rolling direction to the projections formed on the web surface can reduce buckling. In addition, buckling can also be reduced because reduction in the inner web width is carried out with a universal mill while the rolling workpiece is also being rolled with an edging mill or another universal mill on the upstream side, as long as the pass line through the mills is on the same level.
(2) Furthermore, as indicated by arrows in Figures 2a - 2c, when the web width reduction rolling is carried out repeatedly using two universal mills, it is possible to reduce the inner web width by 20% - 50% relative to the dimensions of a workpiece after breakdown rolling. In this case, too, it is advisable to carry out expansion of the web width in the first half of passes while the thickness of a web is relatively large and the temperature of the workpiece is relatively high in order to achieve a large degree of expansion as well as to finish a thin web.

The following are preferred embodiments of the present invention.

Figures 4b, 4c and 4d are schematic illustrations of roll mill arrangements for producing H-shaped steels. The present invention will be further described with respect to the roll mill arrangement shown in Figure 4b.

The roll mills employed in this embodiment are schematically shown in Figure 11, in which horizontal rolls divided into two or three pieces are installed in the first universal roughing mill (UR1), edging mill (e), the second universal roughing mill (UR2), and universal finishing mill (UF). The widths of these horizontal rolls can be varied in the axial directions of the rolls for each pass.

Breakdown rolling is carried out in a conventional manner to provide a beam blank, i.e., a rough-rolled workpiece. The beam blank is then subjected to an intermediate rolling step in which reverse rolling is carried out using the universal roughing mills and edging mill arranged in a pattern UR1-E-UR2. The rolling workpiece is rolled to give finished sizes for flange width, inner web width, flange thickness, and web thickness.

According to the present invention, before the intermediate rolling, it is determined whether the web width is to be expanded or reduced or maintained, and then rolling with each of the mills is continued in accordance with a predetermined rolling schedule depending on whether the web height should be expanded, or reduced, or maintained.

A rolling process in which the web height is expanded will next be explained.

As shown in Figure 1a or 1b, during the reduction in web thickness as well as the reduction in the thickness of flanges 1 with one of the universal mills, one or more non-rolled portions 2a are formed on the surface of the web. In the following rolling pass with the other universal mill, not only reduction in thickness of the flange as well as reduction in thickness of the web are carried out to flatten the web surface. Simultaneously, expansion of the web width, i.e., Wa1 < Wa2 or Wb1 < Wb2, is carried out. This process of forming the non-rolled portion and of expanding the width is repeated until a predetermined amount of expansion is obtained.

Next, a rolling process in which the web height is reduced will be explained.

As shown in Figure 2a or 2b, the flattening of the web surface as well as the reduction in the thickness of flanges with one of the universal mills are carried out. In the following rolling pass with the other universal mill, reduction in thickness of the flange as well as reduction in thickness of the web are carried out, and one or more non-rolled portions 2a are formed on the surface of the web. Simultaneously, reduction in the inner web width, i.e., Wa1 > Wa2 or Wb1 > Wb2, is carried out. This process of flattening the web surface and forming the non-rolled portion as well as reducing the web width is repeated until a predetermined amount of reduction is obtained. However, if the non-rolled portion is left on the web surface after the final pass of this intermediate rolling, sometimes it is rather difficult to flatten the web surface even in the universal finishing rolling. Thus, it is desirable that the reduction in the inner web width not be carried out in the final pass of the intermediate rolling.

Furthermore, when it is desirable that the inner web width of the final product be substantially the same as that of a beam blank after breakdown rolling, the roll widths of the horizontal rolls of the first and second universal roughing mills are adjusted to be the same, and only the reduction in the thickness of the flanges and web is carried out, and expansion or reduction of the inner web width is not carried out. Alternatively, rolling for expansion and reduction of the inner web width may be carried out repeatedly one after another.

In the foregoing, the horizontal rolls employed in the first and second universal roughing mills have the configurations shown in Figure 11. The horizontal rolls may also have the configurations shown in Figure 12. In the latter case, the process of expanding or reducing the inner web width is the same as shown in Figures 1c and 2c.

An edging mill may also have variable-width edging rolls, and the width can be adjusted in conformity with that of the horizontal rolls of a universal mill in the preceding rolling step after each of the passes through the preceding mill.

As a final stage of rolling, a workpiece is subjected to final finishing rolling in which the flange angle and thickness of the flanges and web are finished with the universal mill to provide a final product.

According to another embodiment of the present invention, an intermediate rolling and finishing rolling are carried out using a rolling mill arrangement as shown in Figure 4c, in which the horizontal rolls of the universal roughing mill, edging mill, and universal finishing mill are divided in the axial direction, and the width thereof is adjustable before or after each pass. Since the taper angle of the horizontal rolls of the second universal mill is adjusted to be substantially zero, the universal mill serves as a finishing mill. Thus, except for the final pass of the intermediate rolling through UR-E-UF, expansion or reduction in the inner web height can be achieved in the same manner as when using the before-mentioned rolling mill arrangement UR1-E-UR2. In the final pass through the UF mill following the intermediate rolling, the flange angle is corrected and the thickness of the flanges and web is adjusted slightly to meet specifications and obtain a final product.

According to still another embodiment of the present invention, an intermediate rolling and finishing rolling are carried out using a rolling mill arrangement as shown in Figure 4d, in which the horizontal rolls of the universal roughing mills, and edging mills are divided in the axial direction, and the width thereof is adjustable after each pass in an on-line basis.

Namely, in Figure 4d three rolling mill groups U1-E1-U2, U3-E2-U4, and U5-E3-U6, each having three mills, can correspond to the before-described UR1, E, and UR2, respectively, of the rolling mill arrangement UR1-E-UR2. The mill structure of each of the mills is like that shown in Figure 11 or 12.

In this embodiment, too, a rolling process such as shown in Figure 1 or 2 may be performed so as to effect expansion or reduction of the inner web width. In the final pass through the U7 mill, the flange angle is corrected and the thickness of flanges and web is adjusted slightly to meet specifications and obtain a final product.

In this embodiment, another rolling line other than that shown in Figure 4d may be employed. Namely, a plurality of groups of rolling mills, each including a universal mill and edging mill, arranged in a tandem line may be used for this purpose.

An example of the horizontal roll employed in the present invention, which can be divided in an axial direction, and the inner width of which can be adjusted on line after each pass, may be found in Japanese Unexamined Laid-Open Specification No.60-72603/1985. In addition, the shape of the horizontal roll or the number of pieces into which it is divided are not limited to specific ones as long as the purpose of the present invention can be achieved.

### Example 1

Four series of H-shaped steels (H600X300, H700X300, H800X300, and H900X300) were manufactured in accordance with the first embodiment of the present invention without changing any of rolls including those of a breakdown mill.

In this example, the roll mill arrangement employed is that shown in Figure 4b in which the first universal mill (UR1 mill), the edging mill (E mill), the second universal mill (UR2 mill), and the universal finishing mill (UF mill) have the shapes and dimensions shown in Figure 13.

The grooved rolls of the breakdown mill are those for use in manufacturing the H700X300 series. Thus, for the H600X300 series reduction in the inner web width was effected, for the H800X300 and H900X300 series expansion of the inner web width was effected, and for the H700X300 series the inner web width was kept constant without expansion or reduction throughout the rolling process after breakdown rolling.

Table 1 indicates the inner web width set for each of the horizontal rolls after each pass and the expansion or reduction amounts achieved by each pass of a rolling mill.

For the H600X300 series the web surface was flattened by each pass through the UR1 mill, and reduction was performed by odd numbered passes through the UR2 mill.

For the H800X300 and H900X300 series expansion of the inner web width was performed by odd numbered passes through the UR2 mill and by even numbered passes through the UR1 mill.

After 7 passes of reverse rolling through the UR1-E-UR2 mill line, the thickness of flanges and web was adjusted in the UF mill slightly and the flange was made upright so as to meet specifications for final products.

The resulting H-shaped steels having a series of sizes from H600X300 to H900X300 were free of surface defects such as rolling flaws and scratches, and the dimensions were accurate since the width each of the horizontal rolls was adjusted on line before each pass in accordance with the finished dimensions or wear of the rolls. The rolling yield was also excellent.

In addition, since there were no need of changing rolls so frequently, and usually substantially no changing of rolls, rolling proceeding as well as rolling operations can be done efficiently. The roll inventory was reduced to 1/7 compared with that of the prior art, in which horizontal rolls having 7 different widths and web height in 50 mm pitches for the series of H600X300 to H900X300 were required.

### Example 2

Three series of H-shaped steels (H700X300, H800X300, and H900X300) were manufactured in accordance with the second embodiment of the present invention without changing any of the rolls including those of a breakdown mill.

In this example, the roll mill arrangement employed was that shown in Figure 4c in which the universal mill (UR mill), the edging mill (E mill), and the universal finishing mill (UF mill) had the shapes and dimensions shown in Figure 14.

The grooved rolls of the breakdown mill were those for use in manufacturing the H800X300 series. Thus, for the H700X300 series reduction in the inner web width was effected, for the H900X300 series expansion of the inner web width was effected, and for the H800X300 series the inner web width was kept constant without effecting expansion or reduction throughout the rolling process after breakdown rolling.

Table 2 indicates the inner web width set for each of the horizontal rolls after each pass, and expansion or reduction amounts achieved by each pass of a rolling mill.

For the H700X300 series, the web surface was flattened by each pass through the UR mill, and reduction was performed by odd numbered passes through the UF mill.

For the H900X300 series, expansion of the inner web width was performed by odd numbered passes through the UF mill and by even numbered passes through the UR mill.

After 6 passes of a reverse rolling through the UR-E-UF mill line, the thickness of the flanges and web was slightly adjusted in the 7th final pass through the UF mill and the flange was made upright so as to meet specifications for final products.

The resulting H-shaped steels having a series of sizes from H700X300 to H900X300 were free of surface defects such as rolling flaws and scratches, and the dimensions were accurate since the width of the horizontal rolls was adjusted on line before each pass based on the finished dimensions or wear of the rolls. The rolling yield was also excellent.

In addition, since there were no need of changing rolls so frequently, and usually substantially no changing of rolls, rolling proceeding as well as rolling operations could be done efficiently. The roll inventory was reduced to 1/5 compared with that of the prior art, in which horizontal rolls having 5 different widths and web heights in 50 mm pitches for the series of H700X300 to H900X300 are required.

### Example 3

Three series of H-shaped steels of H300X300, H400X200, and H450X200 were manufactured in accordance with the third embodiment of the present invention without changing any of the rolls including those of a breakdown mill.

In this example, the roll mill arrangement employed was that shown in Figure 4d in which the universal mills (U1 - U7 mills), and the edging mills (E1 - E4 mills) had the shapes and dimensions shown in Figure 15.

The grooved rolls of the breakdown mill were those for use in manufacturing the H400X200 series. Thus, for the H300X300 series reduction in the inner web width was effected, for the H450X200 series expansion of the inner web width was effected, and for the H400X200 series the inner web width was kept constant without effecting expansion or reduction throughout the rolling process after breakdown rolling.

Table 3 indicates the inner web width set for each of the horizontal rolls after each pass and expansion or reduction amounts achieved by each pass of a rolling mill.

For the H300X300 series, the web surface was flattened by each pass through the U1, U3, and U5 mills, and the reduction thereof was performed by each pass through the U2, U4, and U6 mills.

For the H450X200 series, one or more non-rolled portions (projections) were formed on the web surface by each pass through the U1, U3, and U5 mills, and expansion of the inner web width was performed by each pass through the U2, U4, and U6 mills.

In the final pass through the U7 mill, the thickness of the flanges and web were adjusted slightly and the flange was made upright so as to meet specifications for final products.

The resulting H-shaped steels having a series of sizes from H300X300 to H450X200 were free of surface defects such as rolling flaws and scratches, and the dimensions were accurate since the width each of the horizontal rolls was adjusted on line before each pass based on the finished dimensions or wear of the rolls. The rolling yield was also excellent.

In addition, since there were no need of changing rolls so frequently, and usually substantially no changing of rolls, rolling proceeding as well as rolling operations could be done efficiently. The roll inventory was reduced to 1/4 compared with that of the prior art, in which horizontal rolls having 4 different widths and web heights in 50 mm pitches for the series of H300X300 to H450X200 are required.

## Claims

1. A process for manufacturing H-shaped steels comprising performing intermediate rolling including universal roughing rolling and edging rolling on a rolling workpiece having a web and flanges after breakdown rolling to provide a semi-finished H-shaped steel, and performing finishing rolling on the semi-finished H-shaped steel using a universal finishing mill to provide a final product, characterized in that the intermediate rolling is carried out using a first universal roughing mill having a horizontal roll divided into two or more pieces in a roll axis direction, the width of which is adjustable for each pass, an edging mill having a horizontal roll divided into two or more pieces in a roll axis direction, the barrel width of which is adjustable for each pass, a second universal roughing mill having a horizontal roll divided into two or more pieces in a roll axis direction, the width of which is adjustable for each pass, and a universal finishing mill having a horizontal roll divided into two or more pieces in a roll axis direction, the width of which is adjustable for each pass, and that the intermediate rolling comprises a first step of forming one or more non-rolled portions on the surface of the web while carrying out reduction in web thickness as well as reduction in the thickness of flanges with one of the first and second universal roughing mills; a second step of flattening the web surface to expand the inner web width while not only reduction in thickness of the flange but also reduction in thickness of the web are carried out with the other universal roughing mill; and repeating the first and second steps until a predetermined amount of expansion is achieved.

2. A process for manufacturing H-shaped steels comprising performing intermediate rolling including universal roughing rolling and edging rolling on a rolling workpiece having a web and flanges after breakdown rolling to provide a semi-finished H-shaped steel, and performing finishing rolling on the semi-finished H-shaped steel using a universal finishing mill to provide a final product, characterized in that the intermediate rolling is carried out using a first universal roughing mill having a horizontal roll divided into two or more pieces in a roll axis direction, the width of which is adjustable for each pass, an edging mill having a horizontal roll divided into two or more pieces in a roll axis direction, the barrel width of which is adjustable for each pass, a second universal roughing mill having a horizontal roll divided into two or more pieces in a roll axis direction, the width of which is adjustable for each pass, and a universal finishing mill having a horizontal roll divided into two or more pieces in a roll axis direction, the width of which is adjustable for each pass, and that the intermediate rolling comprises a first step of flattening the web surface while performing reduction in flange thickness with one of the first and second universal roughing mills; a second step of forming one or more non-rolled portions on the web surface and simultaneously reducing the inner web width while not only reduction in thickness of the flange but also reduction in thickness of the web are carried out with the other universal roughing mill; and repeating the first and second steps until a predetermined amount of reduction is achieved.

3. A process for manufacturing H-shaped steels comprising performing intermediate rolling including universal roughing rolling and edging rolling on a rolling workpiece having a web and flanges after breakdown rolling to provide a semi-finished H-shaped steel, and performing finishing rolling on the semi-finished H-shaped steel using a universal finishing mill to provide a final product, characterized in that the intermediate rolling is carried out using a universal roughing mill having a horizontal roll divided into two or more pieces in a roll axis direction, the width of which is adjustable for each pass, an edging mill having a horizontal roll divided into two or more pieces in a roll axis direction, the barrel width of which is adjustable for each pass, and a universal finishing mill having a horizontal roll divided into two or more pieces in a roll axis direction, the width of which is adjustable for each pass, the finishing rolling is carried out in the final pass of the universal finishing mill, and that the intermediate rolling comprises a first step of forming one or more non-rolled portions on the surface of the web while performing reduction in web thickness as well as reduction in the thickness of flanges with one of the universal roughing mill and the universal finishing mill; a second step of flattening the web surface to expand the inner web width while not only reduction in thickness of the flange but also reduction in thickness of the web are carried out with the other universal mill; and repeating the first and second steps until a predetermined amount of expansion is achieved.

4. A process for manufacturing H-shaped steels comprising performing intermediate rolling including universal roughing rolling and edging rolling on a rolling workpiece having a web and flanges after breakdown rolling to provide a semi-finished H-shaped steel, and performing finishing rolling on the semi-finished H-shaped steel using a universal finishing mill to provide a final product, characterized in that the intermediate rolling is carried out using a universal roughing mill having a horizontal roll divided into two or more pieces in a roll axis direction, the width of which is adjustable for each pass, an edging mill having a horizontal roll divided into two or more pieces in a roll axis direction, the barrel width of which is adjustable for each pass, and a universal finishing mill having a horizontal roll divided into two or more pieces in a roll axis direction, the width of which is adjustable for each pass, the finishing rolling is carried out in the final pass through the universal finishing mill, and that the intermediate rolling comprises a first step of flattening the web surface while carrying out reduction in flange thickness with one of the universal roughing mill and universal finishing mills; a second step of forming one or more non-rolled portions on the web surface and simultaneously reducing the inner web width while not only reduction in thickness of the flange but also reduction in thickness of the web are carried out with the other universal mill; and repeating the first and second steps until a predetermined amount of reduction is achieved.

5. A process for manufacturing H-shaped steels comprising performing intermediate rolling including universal intermediate rolling and edging rolling on a rolling workpiece having a web and flanges after breakdown rolling to provide a semi-finished H-shaped steel, and performing finishing rolling on the semi-finished H-shaped steel using a universal finishing mill to provide a final product, characterized in that the intermediate rolling is carried out using a plurality of mill groups arranged in a tandem line each including at least a universal intermediate mill having a horizontal roll divided into two or more pieces in a roll axis direction, the width of which is adjustable for each pass, an edging mill having a horizontal roll divided into two or more pieces in a roll axis direction, the barrel width of which is adjustable for each pass, and another universal intermediate mill having a horizontal roll divided into two or more pieces in a roll axis direction, the width of which is adjustable for each pass, the finishing rolling is carried out by a universal finishing mill having a horizontal roll divided into two or more pieces in a roll axis direction, the width of which is adjustable for each pass, and that the intermediate rolling comprises a first step of forming one or more non-rolled portions on the surface of the web while performing reduction in web thickness as well as reduction in the thickness of flanges with one of the universal intermediate mills; a second step of flattening the web surface to expand the inner web width while not only reduction in thickness of the flange but also reduction in thickness of the web are carried out with another universal intermediate mill on the downstream side; and repeating the first and second steps continuously downstream until a predetermined amount of expansion is achieved.

6. A process for manufacturing H-shaped steels comprising performing intermediate rolling including universal intermediate rolling and edging rolling on a rolling workpiece having a web and flanges after breakdown rolling to provide a semi-finished H-shaped steel, and performing finishing rolling on the semi-finished H-shaped steel using a universal finishing mill to provide a final product, characterized in that the intermediate rolling is carried out using a plurality of mill groups arranged in a tandem line each including at least a universal intermediate mill having a horizontal roll divided into two or more pieces in a roll axis direction, the width of which is adjustable for each pass, an edging mill having a horizontal roll divided into two or more pieces in a roll axis direction, the barrel width of which is adjustable for each pass, and another universal intermediate mill having a horizontal roll divided into two or more pieces in a roll axis direction, the width of which is adjustable for each pass, the finishing rolling is carried out by a universal finishing mill having a horizontal roll divided into two or more pieces in a roll axis direction, the width of which is adjustable for each pass, and that the intermediate rolling comprises a first step of flattening the web surface while carrying out reduction in flange thickness with one of the universal intermediate mills; a second step of forming one or more non-rolled portions on the web surface and simultaneously reducing the inner web width while not only reduction in thickness of the flange but also reduction in thickness of the web are carried out with another universal intermediate mill on the downstream side; and repeating the first and second steps continuously downstream until a predetermined amount of reduction is achieved.
